

Nov. 8, 1932.

B. C. GOSS

1,886,394

DENSE OPAQUE SMOKE AND IRRITATING FUME AND GAS PRODUCING CHEMICALS

Filed Feb. 24, 1927



Inventor:  
Byron C. Goss,

Joseph W. Harris

Att'y.

## UNITED STATES PATENT OFFICE

BYRON C. GOSS, OF CLEVELAND, OHIO, ASSIGNOR TO THE LAKE ERIE CHEMICAL COMPANY, A CORPORATION OF OHIO

## DENSE OPAQUE SMOKE AND IRRITATING FUME AND GAS PRODUCING CHEMICALS

Application filed February 24, 1927. Serial No. 170,561.

This invention relates to smoke and fume producing chemicals, and apparatus therefor, the smoke constituting a dense opaque body of gas or vapor that practically obscures vision, and which may be intimately mixed and associated with a gas or vapor of the irritating "tear" or lachrymatory gas type, or similar irritating disabling gas or gases which will produce pain, coughing, sneezing, 10 etc., etc.

An object of the invention is to quickly produce a large volume of dense opaque smoke intimately mixed with an intensely irritating gas, which will disable a bandit 15 when attempting to open a safe, or vault, or to enter a room, or commit other criminal act;

A further object of the invention is to provide a mixture of chemicals which will 20 quickly generate a volume of dense opaque smoke and fume;

A further object is to provide a mixture of chemicals which will generate a volume of mixed smoke and fume, including "tear 25 gases" and similar disabling fumes and gases;

A further object is to provide a mixture of smoke and fume and irritating "tear" gas producing chemicals with a reagent which also generates a fume on reacting with the 30 chemicals, and which by the chemical reaction also supplies heat to vaporize the mixed chemicals;

A further object is to provide an apparatus in which the chemicals and reagent may be 35 retained until ignited, and which will serve as a container or vessel in which the reactions may take place;

A further object is to provide an apparatus which will be retained in the "loaded" 40 condition, and which will be "fired" automatically upon disturbing a "release";

A further object is to provide an apparatus to be actuated by an automatic "release" but which will be controlled by a time clock. 45

Other objects will appear upon reading the specification.

The invention comprises means which when "fired" will quickly produce a large 50 volume of dense opaque smoke that will so obscure vision as to render it impossible for

any one to see objects close to hand, and therefore render it impossible for a bandit to open a vault. The smoke producing chemical mixture is mixed with, or in close proximity to, a chemical or chemicals which are capable 55 of producing large volumes of lachrymatory or "tear" gases, and which latter chemical or chemicals are vaporized by the heat generated by the smoke producing chemicals so that both smoke and tear gas are delivered 60 as mixed gases from the container, and collectively produce an intensely irritating and opaque atmosphere in which it is impossible to see, and to remain.

In the accompanying drawing,

Figure 1 shows a vertical longitudinal section of one form of container or device showing fuse mechanism and chemicals;

Fig. 2 shows a top plan view of Fig. 1;

Fig. 3 is a modification of Fig. 1, showing 70 two inner containers;

Fig. 4 is a view in elevation of a bouchon, or firing mechanism;

Fig. 5 is a view of a fuse and cap;

Fig. 6 shows a vertical longitudinal section 75 of an electric device;

Fig. 7 is a plan top view of Fig. 6; and

Fig. 8 is a view in elevation of a cartridge containing the chemicals to be inserted in the electric device.

In Fig. 1, an outer casing 1 is provided with a lid 2 which after loading, is preferably sealed with varnish, or wax, or similar material. The lid is provided with openings 3, which may be threaded, as at 4, or may be 85 provided with a "bayonet joint" slot, to receive the lug 5, Fig. 4, on the "bouchon" 14, or may be any other type of positive detachable retaining socket.

Within the empty can is first placed a mixture of chemicals 6 which when ignited, will generate the opaque smoke and also produce the lachrymatory fumes. At this upper level 7 of the mass of chemicals is placed a tube or tubes, 8, 8, which may be of paper, or 90 other fibrous material, or may be a casting of a suitable lachrymatory chemical. The tube 8 contains a lower layer 9 of a "fast starter" above which is a layer of lead foil, 10, or similar fusible substance, and above the foil is a 100

- space or pocket 11, within which rests the match head 12. The mass of mixed chemicals is covered with a solid layer 13 of a lachrymatory gas producing chemical which seals 5 the contents and holds the tubes 8—8 in place, the particular chemical 13 used may be similar to that used in the mass of chemicals 6, or it may be different, and may consist of several such chemicals, fused together.
- 10 Within the threaded openings 3 are inserted "bouchons" or firing mechanisms, 14, provided with a tubular stem 15, and a threaded portion 16 to engage the opening 3. The bouchon 14 may be made of metal, and is provided with a "firing pin", or striker, 17, spring actuated, and which when in use is held back by an automatic release, not shown. The bouchon 14 is provided with a recess in the upper part, from the walls of which extend 15 lugs 18, leaving a central space 19, Fig. 2, within which is pressed a percussion cap 20. Before inserting the bouchon 14 in the opening 3, a fuse 21, which may be of the Ensign-Bickford type, and provided with a match 20 head 12, or similar ignitable mass, is inserted in the lower end of the tubular opening in the stem 15 until the end of the fuse reaches the central space 19 in the bouchon 14; the bouchon is then inserted in the opening 3 and 25 the percussion cap 20 is inserted in said space 19, and pressed against the upper end of the fuse 21. In Fig. 1, the striker 17 at the right is shown in the "cocked" position, while at the left it is shown in the "fired" position. As 30 noted above, both strikers 17 are held "cocked" by an automatic release, not shown, which "fires" both together. Two bouchons are shown to insure positive operation, although the device will function with one only.
- 35 In some instances, the chemicals used will be solids, and may be mixed and placed in the container, 1, as at 6; in other instances one or more of the fuming chemicals may be a fluid or a soft pasty mass, and may be retained in a suitable inner container, 22, made of thin glass, gelatin, celluloid, wax, or other easily destructible material, which if of glass, may have a scratch as at 23, to facilitate its destruction. There may be 40 more than one such container 22 as shown in Fig. 3, and each may contain a different chemical, which upon volatilization will produce an irritating suffocating fuming lachrymatory gas commingled with the dense 45 opaque smoke.
- 45 In the electrical modification shown in Fig. 6, a container 30 is provided with a perforated cover 31 and screen 32, and a layer of light-weight paper 43, or of similar material, also a removable bottom 42. An electric match head or fuse 33, is associated with a detonating cap, 34, which is in contact with a quick starting mixture 35, in a destructible casing 40; the latter is in contact with the 50 destructible casing 41 containing chemicals 36, which upon ignition produce the mixed opaque and fuming gases. The casing 41 containing chemicals 36 may or may not also include a receptacle 37 holding a liquid 38, as in Figs. 1 and 3. Upon closing the electric circuit through the wires 39, either automatically as by a burglar alarm system, or by hand-operated devices, or by any other means, the device will be "fired" and destroy 55 the destructible casings, and deliver the generated fuming smoke and gases from the perforated cover 31.
- 60 The chemicals used to generate the dense opaque smoke produce considerable heat by the reaction, vaporizing the resulting products which issue in a dense streaming mass of fume which obscures vision and renders it impossible to see to perform any acts. The chemical mixture used to produce an opaque smoke of this kind may contain zinc 65 dust and hexachlorethane, with or without more or less ammonium perchlorate, zinc oxide, ammonium chloride, or calcium carbonate, or a mixture of them. The speed of the reaction may be increased by an increase in the proportion of ammonium perchlorate, or equivalent chemical, or may be decreased by the increase in the quantity of zinc oxide, ammonium chloride, or calcium carbonate used. The proportions used may vary, but 70 an operative combination will be given below.
- 75 In combination with the smoke generating chemicals, I have found that the heat liberated by the reaction is sufficient to volatilize a lachrymatory gas producing chemical, or a mixture of such chemicals, with the result that I am able to obtain mixed gases which are densely opaque, and also are intensely irritating, causing lachrymation, coughing, sneezing, etc., etc. The irritating gas producing chemicals may be mixed with the smoke producing chemicals, or may be in part mixed therewith and a greater or less quantity placed 80 in a separate container such as thin glass, wax, etc., etc., and embedded in the mass of the smoke producing chemicals. In this latter case, the heat generated by the chemical reaction will destroy the small container and volatilize the liquid or other chemical contained therein, the vapors or gases produced thereby mixing with the dense smoke and producing a mixed mass of densely 85 opaque fuming irritating gas.
- 90 The chemicals producing irritating gases may be solids, liquids, pastes, etc., and may consist of one such chemical, or a suitable mixture of two or more of them. Among solid chemicals suitable for this purpose are chloracetophenone, diphenylamine-chlorarsine, capsaicin, diphenylchlorarsine, bromacetophenone, iodacetophenone, parabromacetophenone, etc. Among liquid chemicals suitable for this purpose are—ethylbromacetate, 95 100

- 10 methylbromacetate, chloracetone, benzylbromide, brombenzalcyanide, ethyliodoacetate, phenylisocyanide, bromacetone, chloromethyl-chloro-formate, chloracetotoluene, phenylcarbylaminechloride, etc. Increased concentration of the lachrymatory gas producing chemicals may be effected by dissolving appropriate solids in appropriate liquids, above enumerated.
- 15 An operative combination of chemicals to produce mixed dense opaque smoke and irritating gases is as follows, but the formula is given as illustrative only, as many variations in percentage and substitutions of the above noted chemicals, in whole or in part, may be made without departing from the scope of the invention:

|                      | Per cent |
|----------------------|----------|
| Hexachlorethane      | about 28 |
| Zinc dust            | about 22 |
| Ammonium perchlorate | about 12 |
| Zinc oxide           | about 8  |
| Chloracetophenone    | about 30 |

- 20 As noted above, substitutions or variations may be made, and in the above formula, capsaicin or diphenylaminechlorarsine may be substituted in whole or in part for the chloracetophenone. Where liquids are used in combination with, or as a substitute for the irritating and lachrymatory chemicals, the liquid or liquids are placed in suitable fragile vessels, as shown.

- 25 A suitable charge for the device shown in Figure 1 is as follows:
- 30 For the quick starting mixture, indicated as 9 in Figure 1, the composition may be

|                      | Grams     |
|----------------------|-----------|
| Hexachlorethane      | about 2.4 |
| Zinc dust            | about 1.9 |
| Zinc oxide           | about 1.0 |
| Ammonium perchlorate | about 0.7 |
|                      | 6.0       |

- 35 For the mass of mixed chemicals to produce the mixed dense smoke and irritating gases, indicated as 6 in Fig. 1, the composition may be

|                      | Grams      |
|----------------------|------------|
| Chloracetophenone    | about 12.5 |
| Hexachlorethane      | about 52.5 |
| Zinc dust            | about 34.0 |
| Zinc oxide           | about 21.5 |
| Ammonium perchlorate | about 4.5  |
|                      | 125.0      |

- 40 In the electric device, shown in Fig. 6, the quick starting composition, indicated as 35, may be the same as described above, indicated as 9 in Fig. 1. The mass of chemicals indicated as 36 in Fig. 6 may consist of

|                   | Per cent   |
|-------------------|------------|
| Chloracetophenone | about 30   |
| Zinc dust         | about 22.4 |

|                      |            |
|----------------------|------------|
| Hexachlorethane      | about 27.3 |
| Zinc oxide           | about 11.9 |
| Ammonium perchlorate | about 8.4  |
|                      | 100.0 70   |

or may be the same as used in the container 1, or may consist of a minor variation of either of these formulas.

Upon firing the match electrically in Fig. 6, or by the striker and percussion cap in Fig. 1, the temperature of the quick-starting composition is raised, and a chemical reaction is induced between the zinc and the hexachlorethane, generating considerable heat and forming the dense opaque smoke compounds above described. The quick-starting composition ignites the principal body of the charge inducing a similar chemical reaction, which also forms greater volumes of dense opaque smoke and also volatilizes the irritating lachrymatory gas producing chemicals, which gas is generated simultaneously with the smoke and is commingled therewith, the combined smoke and gases being delivered together as a large volume of fuming irritating disabling gases and dense opaque smoke.

In use, the device shown in Fig. 1 is placed in a safe or vault, and the strikers held "cocked" by an automatic release, not shown, which is also controlled by a time clock. Upon the opening of the safe or vault at an improper time, as by a bandit, the device is "fired" and the smoke and fume liberated. The electrical device is connected to a suitable electric alarm system, and is also operated either automatically, or manually.

I claim:

1. A disabling and irritating mixed gas and smoke generating composition comprising a mixture containing from about 12.5 percent to about 30 percent of chloracetophenone, from about 27.3 percent to about 52.5 percent of hexachlorethane, and also containing ammonium perchlorate, zinc dust, and zinc oxide.

2. A disabling and irritating mixed gas and smoke generating chemical composition comprising a mixture containing from about 12.5 percent to about 30 percent chloracetophenone, from about 27.3 percent to about 52.5 percent of hexachlorethane and from about 22 percent to about 34 percent of zinc dust.

3. A disabling and irritating mixed gas and smoke generating composition comprising a mixture containing from about 12.5 percent to about 30 percent of chloracetophenone, from about 27.3 percent to about 52.5 percent of hexachlorethane, from about 4.5 percent to about 12 percent of ammonium perchlorate, and also containing zinc dust and zinc oxide.

4. A disabling and irritating mixed gas and smoke generating chemical composition

comprising a mixture containing from about 12.5 percent to about 30 percent chloracetophenone, from about 27.3 percent to about 52.5 percent of hexachlorethane, and from about 22 percent to about 34 percent of zinc dust, and also containing from about 4.5 percent to about 12 percent of ammonium perchlorate.

5. A disabling and irritating mixed gas 10 and smoke generating chemical composition comprising a mixture containing from about 12.5 percent to about 30 percent chloracetophenone, from about 27.3 percent to about 52.5 percent of hexachlorethane, and from about 22 percent to about 34 percent of zinc dust, and also containing from about 4.5 percent to about 12 percent of ammonium perchlorate, and also containing from about 8 percent to about 21.5 percent of zinc oxide.

20 6. A disabling and irritating mixed gas and smoke generating chemical composition comprising a mixture of from about 12.5 percent to about 30 percent of at least one of the chemicals in group A and also containing from about 27.3 percent to about 52.5 percent of hexachlorethane, from about 22 percent to about 34 percent of zinc dust, said group A chemicals consisting of chlorecetophenone, diphenylamine-chlorarsine, capsaicin, diphenylchlorarsine, bromacetophenone, iodacetophenone, parabromacetophenone, ethylbromacetate, methylbromacetate, chloracetone, benzylbromide, brombenzalcyanide, ethyliodoacetate, phenylisocyanide, bromacetone, chloro-methyl-chloro-formate, chloracetotoluene, and phenylcarbiamine-chloride.

7. A disabling and irritating mixed gas and smoke generating chemical composition 40 comprising a mixture of from about 12.5 percent to about 30 percent of at least one of the chemicals in group A, and also containing from about 27.3 percent to about 52.5 percent of hexachlorethane, from about 22 percent to about 34 percent of zinc dust, from about 4.5 percent to about 12 percent of ammonium perchlorate, said group A chemicals consisting of chloracetophenone, diphenylamine-chlorarsine, capsaicin, diphenylchlorarsine, bromacetophenone, iodacetophenone, parabromacetophenone, ethylbromacetate, methylbromacetate, chloracetone, benzylbromide, brombenzalcyanide, ethyliodoacetate, phenylisocyanide, bromacetone, chloro-methyl-chloro-formate, chloracetotoluene, and phenylcarbiamine-chloride.

8. A disabling and irritating mixed gas and smoke generating chemical composition comprising a mixture of from about 12.5 60 percent to about 30 percent of at least one of the chemicals in group A, and also containing from about 27.3 percent to about 52.5 percent of hexachlorethane, from about 22 percent to about 34 percent of zinc dust, from about 4.5 percent to about 12 percent of am-

monium perchlorate, and also containing zinc oxide, said group A chemicals consisting of chloracetophenone, diphenylamine-chlorarsine, capsaicin, diphenylchlorarsine, bromacetophenone, iodacetophenone, parabromacetophenone, ethylbromacetate, methylbromacetate, chloracetone, benzylbromide, brombenzalcyanide, ethyliodoacetate, phenylisocyanide, bromacetone, chloro-methyl-chloro-formate, chloracetotoluene, and phenylcarbiaminechloride.

In testimony whereof I hereby affix my signature.

BYRON C. GOSS.

80

85

90

95

100

105